

June 24, 1930.

W. E. TRENT

1,767,778

PROCESS FOR CARBONIZING COAL

Filed Feb. 27, 1925

Fig. 1.



Fig. 2.



Fig. 3.



Inventor

Walter E. Trent

By Charles M. Thomas

Attorney

## UNITED STATES PATENT OFFICE

WALTER EDWIN TRENT, OF NEW YORK, N. Y., ASSIGNOR TO TRENT PROCESS CORPORATION, OF NEW YORK, N. Y., A CORPORATION OF DELAWARE

## PROCESS FOR CARBONIZING COAL

Application filed February 27, 1925. Serial No. 12,129.

The invention relates to a process for carbonizing coal and coal and oil mixtures to produce carbonized or coked products of substantially the same dimensions as the green preformed fuel masses.

In the treatment of mixtures of coals and oil I have found that if a preformed mass of green fuel is subjected to a heat treatment of a comparatively low temperature for a definite period of time, while in the presence of a slight amount of oxygen, and thereafter subjected to a second stage treatment in a zone maintained at a carbonizing or coking temperature in which little or no oxygen is present, the carbonized or coked product will be free of substantial swelling or shrinkage, and, therefore, of dimensions substantially the same as the dimensions of the original green mass from which the carbonized fuel is produced.

My invention, therefore, broadly comprehends a two-stage treatment in the carbonization of coals, in which the coal in the first stage is partially carbonized under a low temperature in the presence of a limited amount of oxygen and in the second stage is heated to a high temperature in an atmosphere substantially free of oxygen to form the carbonized products herein referred to.

In the accompanying drawings,—

Figure 1 is a view of an apparatus capable of carrying out the first-stage treatment; and

Fig. 2 is a view of the apparatus used in the second-stage treatment of the coal.

Fig. 3 is a view of a slightly modified form of pan.

Referring now more particularly to the drawings, wherein like reference characters indicate corresponding parts, the numeral 1 designates the carbonizing furnace used for the purpose of heating the material to a low temperature in the presence of oxygen. This furnace has a sprocket 2 at one end and is also provided with gas outlet pipes 3 leading to a header 4. A sprocket 5 is disposed outside of the furnace and this sprocket together with the sprocket 2 receives the endless conveyor 6 carrying a

series of pans 7 each having a false bottom 8, providing a receiver 9 for heat storage elements to be later described. The pans move through openings 10<sup>a</sup> in one wall of the chamber 1, which openings are sufficiently large to permit the introduction of a limited quantity of oxygen to the chamber 1 during the distillation and heat treatment of the materials therein.

The pans as they reach the point *x* are adapted to each receive preformed masses *a* of coal and oil of a plastic consistency or masses of coal with any suitable binder. These masses may be shaped in a molding machine or other suitable type of apparatus. They are placed in the pan 7 as the pans enter the retort 1. The fuel masses are heated during passage through the retort by heat imparted thereto by heat storage elements 10. These elements are composed of cast iron or other material capable of absorbing heat and are heated in a furnace exteriorly of the oven 1. They are inserted in the pockets 9 formed in each pan at the point *x* and travel with the pans through the carbonizing zone 1, applying heat to the preformed masses in the pans during this travel. As shown in Fig. 3, the pans need not have the false bottom 8. In this operation the heat storing elements 10 rest on the bottoms of the pans and the preformed masses seat directly on these elements.

When a pan reaches the point *x* the cool heat storing member 10 is removed and a heated element substituted in its place. One or more of the preformed masses *a* are then placed in the pan. The pan with its heat storing element passes on through the carbonizing retort undergoing a low temperature carbonizing treatment therein in the presence of oxygen entering the retort through the openings 10<sup>a</sup>. In this operation the heat storing elements 10 are preferably heated to a temperature sufficient to impart to the preformed fuel masses a temperature of from 450 to 575° F. The speed of the conveyor through the retort is regulated so that it will require from 45 minutes to 1 hour 30 minutes for a pan with its material to travel through the retort to the

sprocket 2. This temperature and time of treatment is followed when using a non-coking coal. If a highly coking coal is used, substantially the same temperatures are employed but the time of treatment must be longer. This time of treatment will vary from one and one-half hours to four hours. The coal thus treated will be hardened or carbonized around its surface but will not be coked. The fuel masses may be said to be no more than case-hardened by this treatment, and of course, a substantial quantity of the lighter volatiles is removed.

After treatment in the retort 1 the case-hardened fuel masses are dropped into the trough 11 and discharged through the outlet line 12 on to a conveyor 13, the empty receivers passing on back to the point *x* where new heat storage elements are inserted and where fresh charges of fuel are placed in the receivers.

The foregoing treatment constitutes the first-stage treatment of the fuel.

The case-hardened masses depositing on the belt 13 are then led by this belt to a suitable retort 14 where said masses are subjected to a considerably higher temperature to undergo a higher degree carbonization therein. Various forms of retorts can be used for this purpose but for the sake of illustrating the invention I have disclosed a vertical shale retort. This retort has an outer insulated wall 15 and an inner spaced wall 16. The lower part of the wall 16 is lined with fire clay 17 while the upper portion thereof consists merely of steel or iron, there being a space 18 between the walls. The carbonized fuel masses carried by the belt 13 are discharged into the hopper 19 at the top of the retort and permitted to enter the retort by the opening of the valve 20. These masses fill the retort which has its lower end closed by a belt 21 movable over pulleys 22. Gas burners 23 enter the space 18 between the walls of the retort, producing a flame that is projected against the wall 16 of the retort, raising the temperature thereof to the desired degree. I preferably heat the carbonized masses in the retort at a temperature of from 1100 to 1200° F. This maximum temperature is attained near the lower part of the retort. Little or no air is present in the interior of the retort containing the pre-formed fuel masses 24 which are undergoing heat treatment therein, and I have discovered that when these masses are treated in this retort under the temperatures mentioned in the absence of air, that the case-hardened masses will carbonize or coke without swelling. That is to say, the carbonized fuel thus produced is in the form of pre-formed masses of the same dimensions as the dimensions of the green fuel charges introduced to the preheating or case-hardening retort 1. There is no swelling nor

shrinkage of these fuel masses during treatment. The gases driven from the fuel charges in the retort pass through the gas and vapor line 25 to a point of condensation and collection.

It will be observed that in the bottom of the retort I provide steam jets 26. Steam issues from these jets, serving to quench the treated preformed carbonized masses and to also drive heat away from the wall 16 near its bottom and to carry this heat into the carbonized masses of fuel in the retort. This steam, therefore, acts as an agent to prevent over-heating of the brick wall 17 of the wall 16 and to distribute heat throughout the retort.

The bottom walls of the retort are slightly cut away as indicated by the reference character 27 and as the fuel masses reach the bottom of the retort the conveyor 21 is moved to carry out of the retort those masses that have been sufficiently treated. Such masses are led to a point of collection.

In treating the case-hardened masses in the final retort I preferably subject such masses to a treatment of from 45 minutes to one and one-half hours, and as before stated, heat the carbonized masses to a temperature of from 1100 to 1200° F. This, I have found, causes a complete carbonization or coking of the fuel charges without causing these charges to swell or become distorted. It will also be observed that this high temperature treatment should be carried out in an atmosphere in which little or no oxygen is present.

It is believed from the foregoing that the operation of this process is apparent but it may be briefly repeated as follows:

Fuel masses formed in a molding machine, press or the like, of any desired contour, are placed in the pans 7 which also carry the heat absorbing elements 10. These fuel masses *a* pass through the low temperature oven 1 and undergo partial carbonization in the presence of oxygen admitted to said retort through the openings 10<sup>a</sup>. This treatment causes a case-hardening or partial carbonization of the fuel masses. They are discharged from the containers as the containers pass around the sprockets 2, are deposited on the belt 13 and led to the high temperature retort 14. In this retort 14 a temperature of from 1100 to 1200° F. is maintained as compared with the comparatively low temperature of from 450 to 575° F. in the retort 1. Little or no oxygen is permitted to enter the retort 14 and the coking or carbonizing of the partially carbonized masses entering this retort is carried on in the absence of an oxidizing atmosphere. A definite time of treatment must be maintained in the low temperature retort 1 and also in the high temperature retort 14. These periods of treatment have heretofore been set forth.

The fuel masses discharging from the retort 14 are substantially completely carbonized and these masses are neither swollen nor has there been any substantial shrinkage as compared with the original fuel masses *a*. The 5 carbonized product recovered is of dimensions substantially the same as the dimensions of the green fuel charges from which the product is made. These fuel charges are carried from the retort 14 by the belt 21 10 trained around pulleys 22 and deposited in a suitable storage space or container not shown.

Having thus described the invention, what I claim is:

15 1. A carbonizing process, consisting in applying preformed masses of carbonaceous material of at least plastic consistency to a receiver, in disposing in heat conductive relation with said masses heat storage elements, 20 in moving the fuel masses and heat storage elements through a retort where the fuel masses are heated to a temperature in the presence of air sufficient to partially carbonize the same, in then transferring the partially carbonized fuel masses to a second retort, and in subjecting said masses in said retort to a substantially increased temperature while in an atmosphere largely free of 25 oxygen for such time as to completely carbonize the fuel masses without causing distortion or shrinkage thereof.

2. A process for carbonizing preformed masses of carbonaceous material of at least plastic consistency, consisting in preliminarily introducing said masses to a heating zone, in there heating the masses to a temperature sufficient to cause only partial carbonization thereof while permitting a free unobstructed 35 entrance of air to said preliminary heating zone, in introducing the partially carbonized fuel masses to a final heating zone, in subjecting said masses in said zone to a substantially higher temperature for such time as to 40 completely carbonize the fuel masses without causing distortion or shrinkage thereof while substantially excluding air from said final heating zone, the initial heat treatment of the fuel masses being characterized by the 45 application of heat to said masses transmitted thereto by heat storage elements containing sufficient heat to partially carbonize said masses.

3. A process of carbonizing preformed 55 masses of carbonaceous material of at least plastic consistency consisting in introducing said preformed masses to a preliminary heating zone, in moving said masses through said zone while positioned adjacent heat 60 storage means having storage capacity sufficient to partially carbonize said masses by the contained heat thereof, in permitting a free admission of air through said zone during the carbonization of materials therein, 65 in subjecting the partially carbonized masses

to an increased temperature in a final heating zone to complete carbonization thereof while excluding air from said zone.

In testimony whereof I affix my signature.

WALTER EDWIN TRENT. 70